

## UNITED STATES PATENT OFFICE

VAMAN R. KOKATNUR, OF NEW YORK, N. Y.

## MANUFACTURE OF EMBROIDERY, LACE, AND SIMILAR ARTISTIC PRODUCTS

No Drawing.

Application filed May 27, 1925. Serial No. 33,290.

My invention relates to the manufacture of embroidery by stitching a certain design with a naturally inert thread on a cloth backing consisting of a material which is particularly soluble or sensitive to attack and subsequently removing the said backing by dissolution or by disintegration. Thus in the manufacture of embroidery the idea of dissolving out the backing leaving the embroidery intact, is not new. But heretofore the choice of a suitable backing that can be dissolved out from its embroidery by agents that would not damage the latter, has been a matter of difficulty as well as expense greatly hampering the choice embroidery materials. Thus in making cotton embroidery, fabric-backs of wool, silk, or even rubber had to be used. When the embroidery is stitched on a woolen backing and the whole is subsequently put in a bleaching bath of calcium hypochloride, the woolen back is disintegrated by the action of hypochloride, leaving the embroidery intact and bleached. When rubber is used as a backing, it is removed from the embroidery by dissolution in organic solvents. In such processes the backing is usually more expensive than the embroidery material. Heretofore no one has so far as I know been able to use successfully a cheaper backing of cotton or jute in the manufacture of embroidery without giving the same a preliminary treatment such as with oxalic acid, that was in danger of communicating itself to the cotton and injuring the embroidery. To remove cotton or vegetable fibre backing from cotton stitched embroidery has appeared quite impossible and no attempt seems to have been directed towards the solution of this problem.

To treat the fabric-back chemically in some way so that it would behave differently toward certain reagents, than the embroidery, may appear quite logical. But the vegetable fibre does not lend itself to such treatments without operations that are quite technical, expensive and sometimes dangerous. Thus nitration or esterification of the backing might suggest itself; but in either case, the process becomes rather difficult and technical. Also without question, it is expensive if not

dangerous. In addition to the aforementioned difficulties, there has not been found heretofore any chemical reagent that, while destroying one of the fibers, will not harm in any degree the other fiber. Thus in dealing with a vegetable and animal fiber combination, the solvents of the one (for example caustic or strong bleaching solution if the animal fiber is to be destroyed) also attack, though in a minor degree, the other fiber. 55 60

I have found that I can bring about a better result in a simple and relatively inexpensive way and without the least possible danger either to the embroidery or to the operations, by suitably protecting my embroidery thread to prevent its destruction instead of treating the backing to promote its destruction and then subsequently removing the backing by solution by any "reagent" such as well-known vegetable-fibre solvents or disintegrating agents already known, or specially prepared for this purpose. Thus I may treat the fibre or thread to be used in the embroidery either with wax, or oil, or rubber, or the plastic compounds or synthetic resins, or with aluminum oleate or any substance which protects it from the action of the reagent either by preventing the penetration of the agent, by neutralizing its action or by repelling the solvent in which it is dispersed as for example aluminum oleate repels water in which oxalic acid might be dissolved. I further illustrate my invention by the following examples:— 70 75 80 85

*Example I*

I take the usual commercial embroidery yarn of cotton and dip it for a short time in any melted wax or a solution of such waxy materials. I prefer to use an inert wax of a high melting point which is not reacted upon by the usual vegetable fibre solvents. High melting paraffin wax with or without the admixture of other waxy materials to improve its qualities, is suitable for this purpose. I may, however, use any waxy-material whether truly inert or not, as long as it lends itself to substantially protecting the fibre. Thus beeswax, various water-insoluble gum-resins, chlorinated waxes from naphtha- 90 95 100

line and other organic substances and even some fatty acids may be useful depending upon the solvents used later to dissolve out the backing. When using a waxy solution, I 5 may choose a non-combustible organic solvent of suitable volatility, e. g. carbontetrachloride, trichlorethylene. I now use this wax-protected thread for stitching embroidery on any cotton cloth. I then subject the em- 10 broidered back to the action of concentrated hydrochloric acid for a few minutes and after removing the acid by pressing and not wash- 15 ing, I dry the whole at a suitable temperature, or I may treat it with concentrated hydrochloric acid in which free chlorine or hy- 20 pochlorous acid is dissolved when the back is dissolved out in the cold just by immersion. The dried back in the former case is brittle and can be crumpled and brushed off from 25 the embroidery which has not been touched by hydrochloric acid. The wax from the embroidery may be dissolved and recovered for using over and over again. In this example I may use fatty acid protector for the em- 30 broidered back as it is not affected by hydro- 35 chloric acid in which it is insoluble. I may also use jute or other vegetable fabrics as backing.

*Example II*

30 Everything same as in Example I except that I may treat the embroidered back with a saturated solution of zinc-chloride or zinc-chloride and hydrochloric acid as a solvent.

*Example III*

35 The treatment before embroidery stitching being the same as in Example I, I treat the embroidered back with strong sulphuric acid alone or with a suitable mixture of sulphuric and nitric acids in such a way as to 40 tender the back and dissolve it out.

*Example IV*

45 The preliminary treatment of the yarn and stitching the embroidery being the same as in Example I, I then treat the embroidered back with a solution of cuprammonium and dissolve out the back from the embroidery.

*Example V*

50 All else same as in Example I except that I subsequently treat the embroidered back with strong caustic soda solution to the mer- 55 cerizing point and then add enough carbon bi-sulphide to dissolve out the back and wax in one operation.

To particularize: Stitch an embroidery design with wax-protected thread on any 60 cotton foundation. Dip this embroidered cloth in caustic soda solution and without removing the caustic soda, treat it with carbon bi-sulphide. The reason why carbon bi- 65 sulphide does not dissolve out the embroidery is as follows: The wax-protected embroidery

does not absorb caustic soda as wax is inert to caustic and water-resistant. The caustic is absorbed by the foundation cloth only. The carbon bi-sulphide forms xanthate when it comes in contact with caustic-soaked foun- 70 dation and dissolves it out. It does not touch the embroidery as it has no caustic and hence no xanthate is formed on its surface.

I do not wish to limit myself to these five examples as they are only of illustrative na- 75 ture. In carrying out my invention, I may protect the embroidery yarn with any mate- 80 rial, substantially inert under the conditions used and insoluble in the particular solvent or solvents used later on to dissolve out the back. I may prefer to make the yarn pliable by first dipping it in high boiling oils such as lubricating oils or drying or non-drying fatty oils and after pressing out the said oil, may further treat it with a solution of a mix- 85 ture of waxy materials. Thus I may em- 90 broider with silk, artificial silk, wool or any vegetable fibre or union (mixed fibre) yarn or cotton, jute or any cheap vegetable fabric and dissolve out or disintegrate the back 95 from the embroidery. It is understood that I may utilize the various dissolved out solu- 100 tions of vegetable-fabric backs in various arts as by-products such as fibre-board, vul- 105 canized fibres, artificial silks, collodions, var- 110 nishes and in plastics.

Having thus fully described my invention, what I claim is:

1. The process of manufacturing embroi- 100 deries or laces which comprises treating the embroidery yarn with a coating of a mate- 105 rial which is pliable and inert to solvents of the yarn fibers, stitching the yarn upon a base fabric composed of the same fiber as the em- 110 broidery yarn and discharging the base fab- 115 ric by means of such solvents.

2. The process of manufacturing embroi- 110 deries or laces which comprises treating the embroidery yarn with a coating of waxy ma- 115 terial, stitching the yarn upon a base fab- 120 ric composed of the same fiber as the embroidery yarn and discharging the base fabric by means of solvents of such fiber.

3. The process of manufacturing embroi- 115 deries or laces which comprises treating the embroidery yarn with a coating of a material which is pliable and inert to discharging 120 agents for the embroidery yarn fibers, stitching the yarn upon a base fabric composed of the same fibers as the yarn and discharging the base fabric by means of such discharging agents.

VAMAN R. KOKATNUR.